

## UNITED STATES PATENT OFFICE

2,448,753

HEAT-TREATING AND COLD-ROLLING  
HADFIELD MANGANESE STEEL

Carl W. Weesner, Warren, Ohio, and Wallace B. Leffingwell, Sharon, Elvan R. Babylon, New Wilmington, and Homer L. Schell, Sharon, Pa., assignors to Sharon Steel Corporation, Sharon, Pa., a corporation of Pennsylvania

No Drawing. Application December 16, 1943,  
Serial No. 514,548

10 Claims. (Cl. 148—12)

1

The invention relates to the manufacture of manganese steel strips and the like, and more particularly to the manufacture of thin gauge, cold rolled, high manganese, high carbon steel strips and the like adapted to be used among other purposes for making helmets for the armed forces.

Helmet steel must be soft, ductile and have deep drawing qualities in order that helmets may be properly formed or drawn to the desired shape from high manganese steel. High manganese or "Hadfield" steel, that is, steel containing from 10% to 20% manganese and from 1.00% to 1.50% carbon as thin as .044 to .033 inch, and cold rolled and heat treated is admirably suited for such purposes. However, extreme difficulties have been encountered and considerable damaged or scrap material has been made in attempts to manufacture such material.

Some of these difficulties and what is believed to be the explanation of the causes of the same are set forth in the copending Weesner and Leffingwell applications which have matured as Patents Nos. 2,368,955 and 2,410,322. However, the inventions described in said Weesner and Leffingwell patents are directed more particularly to ways and means of reclaiming or salvaging such damaged high manganese strip material.

The present invention involves the avoidance or elimination of the conditions which apparently cause the material to be damaged during the cold rolling and heat treatment thereof. Thus, the difficulties or damage apparently are caused in part by surface embrittlement resulting from decarburization.

In our early attempts at cold rolling and heat treating Hadfield strip two conditions were found associated with low ductility—first, carbide precipitation at grain boundaries, and, second, "frosty" surface, i. e. the frosty appearance resulting from innumerable small cracks developed by the Olsen ductility cup test.

We discovered that the carbide precipitation difficulties could be controlled by a very careful control of the cooling or quenching stage of the heat treatment step.

Tests made revealed that the frosty surface was accompanied by decarburization. Samples known to be frosty and decarburized were recarburized and heat treated very carefully under controlled laboratory conditions and then tested. After the recarburizing heat treatment, the frosty condition disappeared and the ductility as determined by the Olsen cup test, was materially increased. Thus, it was finally determined that

2

the "frosty" surface embrittlement is the result of decarburization.

In most steels, lowering the carbon content tends toward softness and ductility, but Hadfield steel behaves in a contrary manner. The ductility of Hadfield steel when present is due to its austenitic composition. When the carbon content is considerably lowered, the high manganese austenite is no longer stable on cooling, but tends to decompose, probably forming a brittle mixture of epsilon and alpha iron.

Unfortunately, it is hardly possible and not practical in the commercial manufacture of thin gauge high manganese, high carbon strip steel to recarburize material which has become decarburized, in order to correct the conditions found to exist, as shown by recarburization of samples in laboratory tests; so it became absolutely essential to find some way in which the decarburization during heat treatment could be eliminated.

The normal heat treating cycle for Hadfield steels includes heating the steel to a temperature above the upper critical point, approximately 1800° F. to 1900° F. and usually about 1850° F., and then quickly cooling the same, as set forth in said Weesner and Leffingwell patents.

We have discovered that Hadfield steel responds to heat treatment extremely rapidly and that the steel is completely austenitized almost instantaneously upon being heated to a high temperature of from 1900° F. to 2000° F. and preferably from 1950° F. to 2000° F. in a furnace in which the temperature is maintained in the hottest zone at approximately 2000° F.; and these furnace and steel temperatures are materially higher than those previously used for heat treating Hadfield steels.

We have further discovered that the extent of decarburization occurring in Hadfield steel which is the cause of the difficulties, is proportional to time and that if the steel is substantially instantaneously completely austenitized by extremely rapid heating to the high temperature of from 1900° F. to 2000° F. and then immediately quenched, insufficient time elapses for any appreciable amount of decarburization to occur. It is therefore possible by heating and quenching at high speeds, that is by carefully controlling the time and temperature of heating, to hold surface decarburization of Hadfield steel to such a minimum that no harmful effects result.

We have further discovered that the surface appearance of cold rolled heat treated Hadfield steel is no reliable index as to the presence or absence of surface decarburization or embrittle-

ment. If the heat treatment is carried out in a highly oxidizing atmosphere, there is a tendency to scale and "burn" the surface of the Hadfield steel strip at the same time that the decarburization and surface embrittlement occurs. Continued heating of Hadfield steel in a non-oxidizing neutral or moderately reducing atmosphere will produce a decarburized and brittle surface without appreciable scaling or marring of the surface. Thus, a good surface does not necessarily indicate good ductility or the absence of decarburization and surface embrittlement. Continued heating in a very reducing atmosphere, however, produces very little surface decarburization.

Test samples made in the laboratory from the same material were heated for 5 minutes at 1950° F. in three different atmospheres, water quenched and tested. The first sample was heated in a highly oxidizing atmosphere and when tested had a .390 Olsen cup test value with a "frosty" condition. The sample also had heavy decarburization with a rough surface, burned and scaled, and very brittle.

The second sample was heated in a moderately reducing atmosphere. When tested it had a .390 Olsen cup test value with a "frosty" condition. The surface was heavily decarburized and brittle, but the surface appearance was smooth.

The third sample was heated in a very reducing atmosphere and when tested had a .440 Olsen cup test value with no frost. The surface condition was smooth, there was very little decarburization and the sample was ductile.

Therefore, the character of the furnace atmosphere during the heat treatment is also an important factor in addition to the control of the time and temperature of heating. Unfortunately, in mill practice it is not feasible to maintain a highly reducing atmosphere in continuously heating cold rolled Hadfield steel strip as rapidly as it is necessary to do so followed by an immediate quench. For these reasons, it is only possible as a practical matter to control the furnace atmosphere such that it is non-oxidizing, neutral or moderately reducing, which can ordinarily be readily done in the operation of fuel fired continuous heat treating furnaces by a proper control of the burners and of the fuel air ratio. When the furnace atmosphere is thus controlled, and when the heat treating is very rapidly carried out, little if any surface decarburization, burning or scaling occurs.

Accordingly, it is an object of the present invention to provide a method of manufacturing thin gauge, cold rolled, high manganese, high carbon steel strips and the like without surface decarburization or embrittlement, so that the normal ductile properties of austenitic manganese steel may be obtained.

A further object of the present invention is to provide a method of making cold rolled, heat treated, high manganese steel in accordance with strip practice cold rolled to gauges as thin as .044 to .033 inches in thickness.

Furthermore, it is an object of the present invention to provide a new method of manufacturing cold rolled, high manganese steel strips and the like by which the resulting product has a good surface appearance, extreme toughness and strength, and high ductility and drawing qualities.

And finally, it is an object of the present invention to provide a new method of making cold rolled, light gauge, high manganese strip steel 75

and the like more quickly and more cheaply than it has been produced previously.

These and other objects may be obtained, the stated results achieved, and the described difficulties overcome by the methods, steps, products, treatments, and discoveries which comprise the present invention, a preferred outline of the steps being set forth in the following detailed description, and which are particularly and distinctly pointed out and set forth in the claims forming part hereof.

High manganese, high carbon strip steel of the "Hadfield" type is hot rolled down to the thinnest possible gauge to which it can be rolled without damaging the strip or hot mills, which may be approximately .109 inch in thickness, and the strip is then coiled and cooled in water as rapidly as possible to prevent carbide precipitation and decomposition. This cooling step following hot rolling is a departure from usual methods which do not ordinarily include such a step in connection with the manufacture of hot rolled strip.

The hot rolled strip is then continuously heat treated to take the carbides back into solution and to render the steel fully and uniformly austenitic. The heat treatment is performed in accordance with the discoveries of the present invention by substantially instantaneously completely austenitizing the steel by extremely rapid heating to a temperature of from 1900° F. to 2000° F., preferably in the latter half of said range, followed by immediate water quenching.

Thus, the heat treatment of 17 $\frac{1}{2}$ " x .109" and of 15 $\frac{3}{4}$ " x .109" hot rolled "Hadfield" steel has been successfully accomplished in accordance with the present invention in a 25 foot continuous heating furnace in which a non-oxidizing, neutral or moderately reducing atmosphere is maintained, and in which the furnace temperature is maintained at or above approximately 2000° F. The effective interior length of this furnace is approximately 23 feet and the hot rolled strip having the widths and gauge stated have been run at from 9 to 12 feet per minute through the furnace. The strip reaches a temperature close to the furnace temperature of approximately 1950 to 2000° F. at a point approximately 2 feet ahead of the furnace exit opening. The strip is then water quenched as quickly as possible by passing it into a water quenching bath immediately as it leaves the furnace.

As previously pointed out, the cycle of the extremely rapid heating followed by an immediate water quench occurs so quickly that there is no opportunity for surface decarburization of the material to occur.

The strip is then pickled in an inhibited sulphuric acid pickling bath, preferably an aqueous solution of about 10% sulphuric acid by weight in water operated at a temperature of about 150° F.; and the strip is then water sprayed, washed, steam jettied and dried in a hot air drier.

We have also discovered that the pickling step is somewhat critical and particularly the pickling temperature, because "Hadfield" steel burns or pits at a higher pickling temperature and the drying step is necessary to prevent rusting and to eliminate hydrogen for preventing hydrogen embrittlement.

The strip may then be cold rolled from the nominal .109 gauge down to .075 to .080 gauge (31% to 27% reduction, or about 27% reduction) on a four stand tandem cold rolling mill. Other types of cold rolling mills, however, may be used.

The above operations of heating or annealing,

quenching, pickling and cold rolling are then repeated to reduce the strip from .075 to .080 gauge down to .050 to .055 gauge; and again to reduce the strip from .050 to .055 gauge down to .044 to .048 gauge to make the finished cold rolled material; or even again to reduce the strip from .044 to .048 gauge down to .033 to .038 gauge finished material.

The first intermediate anneal after the material has been cold rolled to from .075 to .080 gauge is carried out with a strip speed through the annealing furnace described of about 12 feet per minute; the second intermediate anneal or heat treatment is carried out at a strip speed through the furnace of about 18 feet per minute, the third intermediate anneal is carried out at a strip speed of about 30 feet per minute, and the last intermediate anneal is carried out at a speed of 30 feet per minute or higher.

Thus, in each instance, the heat treatment is carried out in the shortest possible time at the fastest possible rate of heating; and the quench is performed as quickly as possible after leaving the heat treating furnace.

The heat treating operations in each instance are controlled to accomplish several results: first, to recrystallize the cold rolled structure, second, to keep the carbides in solution, and third, to prevent surface decarburization or embrittlement. The heating to the high temperature between 1900° F. and 2000° F. recrystallizes the cold rolled structure, the immediate water quench keeps the carbides in solution, and the rapidity of heating and quenching prevents decarburization. The resulting material is fully and uniformly austenitic with carbides in solution, with the cold rolled structure recrystallized, and without any objectionable decarburized surface layers.

We have discovered that if for some reason the heat treating operation is slowed down, for instance, because of some failure of equipment, or of the necessity of stopping the line for welding one coil to another, thus permitting portions of the strip to lie in the furnace, these portions will have badly decarburized surfaces and these portions must be removed. However, the material therein may be reclaimed by treatment such as described in either of the Weesner and Leffingwell companion patents referred to.

While the process and product have been described in connection with the manufacture of strip steel or stripsheets made in accordance with strip practice, the present invention is also applicable to the manufacture of other high manganese steel products such as sheet steel, in accordance with sheet practice.

Accordingly, when the term "strips" is used herein and in the appended claims, the term is intended to include the manufacture of cold rolled, high manganese steel strips, stripsheets, sheets, wire and the like.

Also, when the term "high manganese steel" is referred to herein, it means steels of the "Hadfield" type, which generally contain from 10% to 20% manganese and from 1% to 1.5% carbon, with possible additions of small percentages of other alloying elements, such as nickel and chromium, which sometimes are added to "Hadfield" steels.

Thus, the present improvements and discoveries provide for the ready and economical manufacture of high manganese steel strips cold rolled to gauges as thin as .044 to .033 inches having extremely high ductility characteristic of

fully austenitic manganese steel; and without surface decarburization or embrittlement.

Having now described the features of the invention; an embodiment of steps by which the invention may be carried out, the advantages and results attained by the invention; and the new discoveries made in connection with the treatment of and cold rolling of high manganese steel; the new and useful methods, steps, treatments, arrangements and products, are set forth in the appended claims.

We claim:

1. The method of producing strong metal sheets of hot-rolled Hadfield manganese steel, which comprises, giving the hot-rolled sheets an austenitizing treatment by heating them to about 1900° F. and water-quenching them and cold-rolling the austenitized sheets to about 27% reduction.
2. The method of making cold rolled Hadfield manganese steel strip, less than 0.109" in thickness, having a fully and uniformly austenitic structure with carbides in solution, and being free of surface decarburization and embrittlement; which comprises, completely austenitizing 0.109" thick hot rolled Hadfield manganese steel strip by heating the strip as it moves continuously through a furnace to a strip temperature of 1900° F. to 2000° F., then before sufficient time has elapsed for the occurrence of surface decarburization quickly water quenching the continuously moving strip immediately as it leaves the furnace to keep the carbides in solution, and then cold rolling the strip down to 0.075" to 0.080" thick strip.
3. The method of making cold rolled Hadfield manganese steel strip, less than 0.109" in thickness, having a fully and uniformly austenitic structure with carbides in solution, and being free of surface decarburization and embrittlement; which comprises, completely austenitizing 0.109" thick hot rolled Hadfield manganese steel strip by heating the strip as it moves continuously through a furnace to a strip temperature of 1900° F. to 2000° F., then before sufficient time has elapsed for the occurrence of surface decarburization quickly water quenching the continuously moving strip immediately as it leaves the furnace to keep the carbides in solution, then cold rolling the strip down to 0.075" to 0.080" thick strip, and then repeating the heating, quenching and cold rolling operations until the strip is reduced to 0.044" to 0.033" thick material.
4. The method of making cold rolled Hadfield manganese steel strip having a fully and uniformly austenitic structure with carbides in solution, and being free of surface decarburization and embrittlement; which comprises, completely austenitizing Hadfield manganese steel strip by extremely rapidly heating the strip as it moves continuously through a furnace to a strip temperature of 1950° F. to 2000° F., then before sufficient time has elapsed for the occurrence of surface decarburization quickly water quenching the continuously moving strip immediately as it leaves the furnace to keep the carbides in solution, and then cold rolling the strip to about 25% reduction.
5. The method of making cold rolled Hadfield manganese steel strip having a fully and uniformly austenitic structure with carbides in solution, and being free of surface decarburization and embrittlement; which comprises, completely austenitizing Hadfield manganese steel strip by extremely rapidly heating the strip as it moves

continuously through a furnace to a strip temperature of 1950° F. to 2000° F., then before sufficient time has elapsed for the occurrence of surface decarburization quickly water quenching the continuously moving strip immediately as it leaves the furnace to keep the carbides in solution, then cold rolling the strip to about 25% reduction, and repeating the heating, quenching and cold rolling operations until the strip is reduced to 0.044" to 0.033" thick material.

6. The method of making cold rolled Hadfield manganese steel strip having a fully and uniformly austenitic structure with carbides in solution, and being free of surface decarburization and embrittlement; which comprises, completely austenitizing Hadfield manganese steel strip by extremely rapidly heating the strip in a non-oxidizing atmosphere as it moves continuously through a furnace to a strip temperature of 1950° F. to 2000° F. to substantially instantaneously obtain complete austenitization of the steel at said temperature, then before sufficient time has elapsed for the occurrence of surface decarburization quickly water quenching the continuously moving strip immediately as it leaves the furnace to keep the carbides in solution, and then cold rolling the strip to about 25% reduction.

7. The method of making cold rolled Hadfield manganese steel strip having a fully and uniformly austenitic structure with carbides in solution, and being free of surface decarburization and embrittlement; which comprises, completely austenitizing Hadfield manganese steel strip by extremely rapidly heating the strip in a non-oxidizing atmosphere as it moves continuously through a furnace to a strip temperature of 1950° F. to 2000° F. to substantially instantaneously obtain complete austenitization of the steel at said temperature, then before sufficient time has elapsed for the occurrence of surface decarburization quickly water quenching the continuously moving strip immediately as it leaves the furnace to keep the carbides in solution, then cold rolling the strip to about 25% reduction, and repeating the heating, quenching and cold rolling operations until the strip is reduced to 0.044" to 0.033" thick material.

8. The method of making cold rolled Hadfield manganese steel strip, less than 0.109" in thickness, having a fully and uniformly austenitic structure with carbides in solution, and being free of surface decarburization and embrittlement; which comprises, completely austenitizing 0.109" thick hot rolled Hadfield manganese steel strip by extremely rapidly heating the strip continuously during 21 feet of strip travel at from 9 to 12 feet per minute in a non-oxidizing atmosphere in a furnace to a strip temperature of 190° F. to 2000° F., then before sufficient time has elapsed for the occurrence of surface decarburization quickly water quenching the continuously moving strip immediately as it leaves the furnace to keep the carbides in solution, and then cold rolling the strip to 0.075" to 0.080" thick strip.

9. The method of making cold rolled Hadfield manganese steel strip having a fully and uniformly austenitic structure with carbides in solution and being free of surface decarburization and embrittlement; which comprises, hot rolling Hadfield manganese steel strip to the thinnest possible hot rolled gauge, then rapidly water cooling the strip, then completely austenitizing the steel by extremely rapidly heating the strip as it moves continuously through a furnace to a strip temperature of 1950° F. to 2000° F., then before sufficient time has elapsed for the occurrence of surface decarburization quickly water quenching the continuously moving strip immediately as it leaves the furnace to keep the carbides in solution, and then cold rolling the strip to about 25% reduction.

10. The method of making cold rolled Hadfield manganese steel strip having a fully and uniformly austenitic structure with carbides in solution and being free of surface decarburization and embrittlement; which comprises, hot rolling Hadfield manganese steel strip to the thinnest possible hot rolled gauge, then rapidly water cooling the strip, then completely austenitizing the steel by extremely rapidly heating the strip as it moves continuously through a furnace to a strip temperature of 1950° F. to 2000° F., then before sufficient time has elapsed for the occurrence of surface decarburization quickly water quenching the continuously moving strip immediately as it leaves the furnace to keep the carbides in solution, and then cold rolling the strip to about 25% reduction.

15. The method of making cold rolled Hadfield manganese steel strip having a fully and uniformly austenitic structure with carbides in solution and being free of surface decarburization and embrittlement; which comprises, hot rolling Hadfield manganese steel strip to the thinnest possible hot rolled gauge, then rapidly water cooling the strip, then completely austenitizing the steel by extremely rapidly heating the strip as it moves continuously through a furnace to a strip temperature of 1950° F. to 2000° F., then before sufficient time has elapsed for the occurrence of surface decarburization quickly water quenching the continuously moving strip immediately as it leaves the furnace to keep the carbides in solution, and then cold rolling the strip to about 25% reduction.

20. The method of making cold rolled Hadfield manganese steel strip having a fully and uniformly austenitic structure with carbides in solution and being free of surface decarburization and embrittlement; which comprises, hot rolling Hadfield manganese steel strip to the thinnest possible hot rolled gauge, then rapidly water cooling the strip, then completely austenitizing the steel by extremely rapidly heating the strip as it moves continuously through a furnace to a strip temperature of 1950° F. to 2000° F., then before sufficient time has elapsed for the occurrence of surface decarburization quickly water quenching the continuously moving strip immediately as it leaves the furnace to keep the carbides in solution, and then cold rolling the strip to about 25% reduction.

25. The method of making cold rolled Hadfield manganese steel strip having a fully and uniformly austenitic structure with carbides in solution and being free of surface decarburization and embrittlement; which comprises, hot rolling Hadfield manganese steel strip to the thinnest possible hot rolled gauge, then rapidly water cooling the strip, then completely austenitizing the steel by extremely rapidly heating the strip as it moves continuously through a furnace to a strip temperature of 1950° F. to 2000° F., then before sufficient time has elapsed for the occurrence of surface decarburization quickly water quenching the continuously moving strip immediately as it leaves the furnace to keep the carbides in solution, and then cold rolling the strip to about 25% reduction.

30. The method of making cold rolled Hadfield manganese steel strip having a fully and uniformly austenitic structure with carbides in solution and being free of surface decarburization and embrittlement; which comprises, hot rolling Hadfield manganese steel strip to the thinnest possible hot rolled gauge, then rapidly water cooling the strip, then completely austenitizing the steel by extremely rapidly heating the strip as it moves continuously through a furnace to a strip temperature of 1950° F. to 2000° F., then before sufficient time has elapsed for the occurrence of surface decarburization quickly water quenching the continuously moving strip immediately as it leaves the furnace to keep the carbides in solution, and then cold rolling the strip to about 25% reduction.

35. The method of making cold rolled Hadfield manganese steel strip having a fully and uniformly austenitic structure with carbides in solution and being free of surface decarburization and embrittlement; which comprises, hot rolling Hadfield manganese steel strip to the thinnest possible hot rolled gauge, then rapidly water cooling the strip, then completely austenitizing the steel by extremely rapidly heating the strip as it moves continuously through a furnace to a strip temperature of 1950° F. to 2000° F., then before sufficient time has elapsed for the occurrence of surface decarburization quickly water quenching the continuously moving strip immediately as it leaves the furnace to keep the carbides in solution, and then cold rolling the strip to about 25% reduction.

CARL W. WEESNER,  
WALLACE B. LEFFINGWELL,  
ELVAN R. BABYLON,  
HOMER L. SCHELL.

#### REFERENCES CITED

The following references are of record in the file of this patent:

#### UNITED STATES PATENTS

| Number       | Name           | Date          |
|--------------|----------------|---------------|
| 938,893      | Potter         | Nov. 2, 1909  |
| 1,017,904    | Potter         | Feb. 20, 1912 |
| 50 1,344,392 | Hadfield       | June 22, 1920 |
| 1,462,460    | Apgar          | July 17, 1923 |
| 1,851,903    | Hall           | Mar. 29, 1932 |
| 1,929,356    | Janitzky       | Oct. 3, 1933  |
| 2,368,955    | Weesner et al. | Feb. 6, 1945  |
| 55 2,378,991 | Franks         | June 26, 1945 |

#### OTHER REFERENCES

- "High Manganese Austenitic Steels," reprinted from "The Iron Age" issue of Oct. 1, 1942, Electro Metallurgical Co., N. Y. C.
- "Alloys of Iron and Chromium," vol. II, Kinzell and Franks, 1940, pp. 289, 438, 442, and 443.
- "Metals Handbook," 1939 ed., pages 1133, 1134, 1135, and 568.